

## UNITED STATES PATENT OFFICE.

JOHN B. FIDLAR, OF BROOKLYN, NEW YORK, AND CHARLES R. FRANKLIN, OF DOVER, NEW JERSEY.

## PROPELLANT POWDER.

No Drawing.

Application filed January 5, 1924. Serial No. 684,650.

(GRANTED UNDER THE ACT OF MARCH 3, 1883; 22 STAT. L. 625.)

*To all whom it may concern:*

Be it known that we, JOHN B. FIDLAR and CHARLES R. FRANKLIN, citizens of the United States, and residents of Brooklyn, in the county of Kings and State of New York, and in Dover, in the county of Morris and State of New Jersey, have invented an Improvement in Propellant Powders, of which the following is a specification.

10 The invention described herein may be used by the Government, or any of its officers or employees in prosecution of work for the Government, or by any other person in the United States, without payment to me of any royalty thereon, in accordance with the act of March 3, 1883.

The subject of the present invention is a propellant powder.

20 The primary object of our invention is the provision of a propellant powder which will meet all ballistic requirements and be flashless and nonhygroscopic.

25 With the foregoing and other objects in view, our invention resides in the novel combination and incorporation of ingredients hereinafter described and claimed, it being understood that changes in the precise embodiment of the invention herein disclosed may be made within the scope of what is claimed without departing from the spirit of the invention.

30 The powder which constitutes the subject of our invention will be made, preferably, from nitrocellulose, nitroglycerine or other similar colloiding explosive, a flash reducing compound and a stabilizer.

35 A powder such as forms the subject of this invention may be made according to the following formula: Nitrocellulose 40 79.5%, nitroglycerine 10.0%, hydrocellulose 10.0%, diphenylamine 0.5%.

40 The formula given above is merely an illustration of some of the materials which may be utilized in the preparation of a propellant powder such as may be manufactured under this invention. Thus for the hydrocellulose, any other flash reducing ingredient such as starch may be substituted, while instead of diphenylamine any other 45 stabilizer of which many are known in the

art, for instance, urea, may be employed. Not only may the ingredients be varied, but the proportions used may be altered within any desired limits.

55 A powder made according to the above formula is especially suitable for use as a propellant in 75 m. m. guns, 155 m. m. Howitzers and other similar arms. It will meet all ballistic requirements, will be 60 flashless and nonhygroscopic. Such a powder may be manufactured according to any suitable process. Methods of manufacture for this and similar powders have been described in the copending applications of C. R. Franklin, Ser. No. 681,629 filed Dec. 19, 1923, and J. B. Fidlar, Ser. No. 520,129 filed December 5, 1921. However, it is not intended to limit our invention to powders manufactured according to the processes described in either of these applications, since 70 the powder which forms the subject of this invention may be prepared by any suitable means.

Having thus described our invention, what we claim is:

1. A propellant powder containing a stabilized mixture of 80 parts, more or less, of nitrocellulose, 10 parts, more or less, of nitroglycerine and 10 parts, more or less, of hydrocellulose.

2. A propellant powder containing a stabilized mixture of nitrocellulose of approximately 12.60% nitrogen content, nitroglycerine, and hydrocellulose.

3. A propellant powder containing a stabilized mixture of nitrocellulose, nitroglycerine, and hydrocellulose.

4. A propellant powder containing a mixture of nitrocellulose, nitroglycerine, and hydrocellulose.

5. A propellant powder containing a mixture of nitrocellulose, a colloiding explosive, hydrocellulose and a stabilizer.

6. A propellant powder containing a mixture of nitrocellulose, a colloiding explosive and hydrocellulose.

7. A propellant powder containing nitrocellulose and hydrocellulose.

JOHN B. FIDLAR.  
CHARLES R. FRANKLIN.